

## UNITED STATES PATENT OFFICE

1,920,857

## DENTAL IMPRESSION MATERIAL

Laurence E. Harrison, Long Beach, Calif., assignor, by mesne assignments, to Dental Plastics Company, Los Angeles, Calif., a Corporation of California

No Drawing. Application June 23, 1930  
Serial No. 463,345

6 Claims. (Cl. 18—47)

This invention relates to a composition of material suitable for use by dentists or dental technicians in making impressions of the teeth and gums. More particularly, the invention relates to a material which is adapted to become plastic upon heating or warming to a certain temperature and to solidify or harden upon again cooling, and which is in other respects particularly adapted for the making of detailed dental impressions and for the subsequent molding or casting of reproductions of the teeth and gums with plaster or other material.

An important object of the invention is to provide a dental impression material which may be removed from the teeth as an integral body, even in cases in which the teeth are disposed at an angle forming undercuts or inverted wedges in the impression, such as are sometimes formed by the extraction of a tooth or a number of teeth and the inward crowding of the adjacent teeth. The principal materials now in common use for this purpose are plaster of Paris, certain waxes, and other substances having similar properties. Such materials, however, are open to the objection that, when in their cooled and solidified state, they are substantially rigid and non-yielding, so that it is often found necessary to break the cast or impression in several places in order to remove it from the mouth and in other cases it is found impossible to remove the cast without completely destroying the impression. In the compound of the present invention these disadvantages are overcome by providing the material with a certain amount of elasticity or resiliency, so as to permit it to give or yield when pulled from the teeth, thus permitting the removal of undercut portions of the impression or of inverted wedges, and to again return or spring back to the original position of the impression after it has been removed.

A further object of the invention is to provide an impression material having yielding or resiliency properties as above mentioned, and being at the same time adapted to soften or become plastic upon warming to a sufficiently low temperature so as not to burn or hurt the mouth of the patient when placed therein, and to again solidify in a relatively short time, upon chilling, sufficiently to retain the exact shape of the impression after its removal from the mouth.

It is also necessary that the material, in order to be useful for the above purpose, shall have certain other properties. Such material must have sufficient body, cohesion, and toughness, so that when squeezed into small crevices and there-

after chilled it will retain its shape, thus enabling the dentist to obtain correct detail and measurements of teeth and of their relation to each other. Furthermore, the material must have the proper contraction upon chilling, in order to permit a correct impression to be obtained.

A further object of the invention is to provide a dental impression material having a pleasant taste and odor, so that the use thereof is not disagreeable to the patient.

The material of my invention comprises, in general, an intimate mixture comprising the following ingredients:

1. Rubber, preferably pure gum rubber or its equivalent. 70  
2. A solid resinous material adapted to soften or flow upon warming to a relatively low temperature (about 35 to 55° C.) and to again solidify upon chilling, such as balata or gutta percha, or both. 75

3. A colloid-forming material, such as gelatine or casein or both.

4. A finely divided solid lubricant material, such as flaked aluminum, or flaked or powdered graphite. 80

The mixture preferably also includes small proportions of glycerol and also of solid oleaginous or waxy material. Such oleaginous or waxy material may comprise a fatty acid, such as stearic acid, which is solid at ordinary temperatures but is adapted to melt at a relatively low temperature, or a paraffin wax which is solid at ordinary temperatures but is adapted to melt at a relatively low temperature, or both a fatty acid and paraffin wax. The composition also preferably comprises a flavoring or scenting material. The above ingredients are intimately mixed together by milling, and properly controlled heating may advantageously be used at certain stages of this operation in order to soften or melt certain ingredients and facilitate the mixing thereof. Furthermore, a small proportion of water is preferably added during the milling process in order to prevent excessive drying of certain of the ingredients and to facilitate the mixing thereof. In general, a portion of this added water remains in the final product, and a portion evaporates off during the mixing operation. The final product, therefore, contains only a very small proportion of water. 105

I have found it advantageous to use certain specific ingredients in certain approximate proportions, as hereinafter described, but it will be understood that the invention in its broader as- 110

pects is not restricted to these specific ingredients and proportions.

The approximate proportions in which the above ingredients are preferably used in making 5 the composition of my invention are as follows:

|                                         | Parts by weight |
|-----------------------------------------|-----------------|
| Rubber                                  | 30 to 50        |
| Fusible resinous material               | 60 to 85        |
| 10 Colloid forming material             | 10 to 30        |
| Finely divided solid lubricant material | 10 to 40        |
| Glycerol                                | 4 to 12         |
| Solid oleaginous or waxy material       | 10 to 20        |

15 To provide the above proportion of resinous material, I may use either balata or gutta percha or combinations thereof. To provide the above proportion of colloid forming material, I may use from 5 to 25 parts of gelatine and from zero to 20 parts of casein or glutin. To provide the above mentioned proportion of solid lubricant material I may use from zero to 20 parts by weight of flaked aluminum and from zero to 40 parts by weight of flaked or powdered graphite. To provide the above mentioned proportion of 25 solid oleaginous or waxy material I may use from 5 to 10 parts by weight of stearic acid and from 5 to 10 parts by weight of paraffin wax. Furthermore, in the making of the material I prefer to add a small proportion of water, say from about 5 to 10 parts by weight, a portion of which may be evaporated during the milling and heating process and a portion of which may remain in the finished material. The material also preferably includes a small amount, say from  $\frac{1}{2}$  to 2 parts by weight, of flavoring and scenting material, such as methyl salicylate.

40 I will now describe a specific embodiment of my invention, using what I consider to be the preferred specific ingredients and the most advantageous approximate proportions thereof, in order to provide a material having the optimum combination of the above mentioned desirable properties. The materials used are as follows:

|                      | Parts by weight |
|----------------------|-----------------|
| Rubber               | 40              |
| Balata               | 72              |
| Gelatine             | 23              |
| 50 Flaked aluminum   | 15              |
| Glycerol             | 9               |
| Stearic acid         | 7               |
| Paraffin wax         | 7               |
| Water                | 7               |
| 55 Methyl salicylate | 1               |

60 The above materials are thoroughly and intimately mixed with one another, preferably by means of milling apparatus such as used, for example, in the milling or compounding of rubber, and the milling operation may be continued for such length of time as is found necessary for this purpose. In general, however, a total milling period of about one hour and thirty minutes is sufficient. Furthermore, the temperature of 65 the mix during the mixing operation may be controlled as by supplying steam or other suitable heating medium, or cold water or other suitable cooling medium, to the rolls or other parts of the milling apparatus.

70 Regarding the substitution of other specific ingredients in the formula given above, it may be said that all or any desired proportion of the balata may be replaced by an equal proportion of gutta percha. However, I find that balata seems to be fully as satisfactory as gutta percha

and is considerably lower in price. The gelatine may be partially replaced by an equal proportion of casein or glutin, but I prefer in any event to use at least five parts of gelatine. Also, in case casein is used in part as the colloid-forming ingredient, I prefer to also add a peptizing agent, such as boric acid, in the proportion of about 1 part of boric acid to 4 parts of casein, and I also prefer in this case to use a somewhat larger proportion of water than would be the case if gelatine alone were used. In case boric acid is used it also acts as an antiseptic or preservative agent in the composition. The flaked aluminum may also be replaced by graphite, but I find that a certain weight of aluminum is more effective as a solid lubricant material than the same weight of graphite, so that the weight of graphite used is preferably about twice as great as the aluminum which is replaced thereby in the above formula. Another advantage of the use of aluminum in preference to graphite is that it has a higher heat conductivity and thus enables the material to be more quickly softened upon heating and to be more quickly solidified to the desired extent throughout, upon chilling.

75 The completed material is solid at ordinary temperatures, but has a certain yielding or resilient property which enables impressions formed therefrom to be removed from the teeth under conditions such as above mentioned, even after 80 chilling to atmospheric temperature or below. At such temperatures, however, the material is not readily susceptible to permanent deformation at ordinary pressures and is adapted to return to its original position when any force causing 85 resilient deformation thereof is removed. The material has a good property of cohesion at all 90 temperatures at which it is to be used and has a satisfactorily tenacious body or consistency which causes it to hold together while making impressions and after removal thereof from the teeth. The material has a fusing or softening point between 35 and 55° C. and preferably between 35 95 and 48° C. (softening temperatures below 48° C. being preferred since they are less apt to cause 100 injury or discomfort to the patient). At these 105 temperatures the material softens and becomes readily plastic and adapted to flow under pressure and fill all recesses, crevices, and small indentations in the teeth and gums when pressed into engagement therewith. A further important property of the material is its ability to chill and solidify quickly throughout after it has been heated to 110 the above temperatures and the impression has 115 been taken. This material in its preferred form has a chilling time, from its fusing or softening 120 temperature to a temperature at which it is adapted to retain its form, of from one to five 125 minutes, upon application of ordinary cold water of about 15 to 30° C. thereto. The material also 130 has a pleasant odor and taste.

135 The method of using this material is, in general, similar to the impression materials now in common use. The material is preferably softened or 140 rendered plastic by placing a quantity thereof in cold water, and bringing the water to a boil in about four or five minutes. The material may then be removed from the water and is sufficiently soft and plastic throughout to permit it to be placed in the usual tray or mold and inserted in 145 the mouth and pressed against the teeth and gums in the usual manner. At the time the material is actually inserted in the mouth, the temperature thereof may be about 45° C. or say between 40 and 50° C. The compound is pressed 150

firmly into contact with the teeth and gums and is then permitted to cool. The cooling may be facilitated by chilling through application of cold water or cold air to the surface of the impression material, and by this means the material may be cooled sufficiently in about one or five minutes to become sufficiently solid for removal of the impression. When the material is in this condition it is sufficiently rigid to prevent permanent deformation or loss of shape, provided ordinary care is exercised in removing the same from the mouth, but is still quite resilient, so that it will yield sufficiently to permit undercut or wedged portions thereof to be readily removed and to then spring back to their original position. Upon further cooling and standing for a period of one hour or more, after removal from the mouth, the material acquires a somewhat more solid and permanent set, so that it may be used for the casting or molding of reproductions in plaster or other material. The material is of such nature as to produce very clean cut reproduction and to produce extremely smooth surface casts in plaster or other material. Even in this state, however, the material has a certain amount of resilience and ability to yield, which properly may be advantageous for certain purposes. For example, this permits the impression to be more easily removed from the cast or reproduction formed therewith, so that the impression may be preserved for further use. Also, it facilitates removal of the impression from the tray or from the plate of an articulator or other apparatus with which it may be used.

35 I claim:

1. A dental impression material consisting principally of rubber and a solid material of a resinous nature similar to balata and adapted to soften upon warming and to solidify upon chilling, said material also comprising a colloid-forming material and a finely divided solid lubricant material, all of said ingredients being intimately mixed together by milling, and said material containing only a very small proportion of water and having a softening temperature between 35 and 55° C.

50

55

60

65

70

75

2. A dental impression material consisting principally of rubber and balata, and also comprising a colloid-forming material and a finely divided solid lubricant material, all of said ingredients being intimately mixed together by milling, and said material containing only a very small proportion of water and having a softening temperature between 35 and 55° C.

3. A dental impression material consisting principally of rubber and balata, and also comprising a colloid-forming material, a finely divided solid lubricant material, glycerol, and waxy material, all of said ingredients being integrally mixed together by milling, and said material containing only a very small proportion of water and having a softening temperature between 35 and 55° C.

4. A dental impression material comprising from 30 to 50 parts by weight of rubber, from 60 to 85 parts by weight of resinous material fusible at a temperature between 35 and 55° C., from 10 to 30 parts by weight of colloid-forming material, from 10 to 40 parts by weight of finely divided solid lubricant material, from 4 to 12 parts by weight of glycerol, from 10 to 20 parts by weight of solid oleaginous material, and less than 10 parts by weight of water.

5. A dental impression material comprising 40 parts by weight of rubber, 72 parts by weight of balata, 23 parts by weight of gelatine, 15 parts by weight of flaked aluminum, 9 parts by weight of glycerol, 7 parts by weight of stearic acid, 7 parts by weight of paraffin wax, 7 parts by weight of water, and 1 part by weight of methyl salicylate, all of said proportions being approximate.

6. A dental impression material comprising from 30 to 50 parts by weight of rubber, from 60 to 85 parts by weight of balata, from 10 to 30 parts by weight of colloid-forming material, from 10 to 40 parts by weight of finely divided solid lubricant material, and less than 10 parts by weight of water.

LAURENCE E. HARRISON.

80

85

90

95

100

105

110

115

120

125

130

135

140

145

150